

Jan. 29, 1974

G. D. MacKENZIE

3,788,997

RESISTANCE MATERIAL AND ELECTRICAL RESISTOR MADE THEREFROM

Filed Dec. 17, 1971



INVENTOR  
GEORGE D. MAC KENZIE  
BY

*Jacob Trachtman*  
ATTORNEY

1

3,788,997  
**RESISTANCE MATERIAL AND ELECTRICAL  
RESISTOR MADE THEREFROM**  
George D. MacKenzie, Maple Glen, Pa., assignor to  
TRW, Inc., Cleveland, Ohio  
Filed Dec. 17, 1971, Ser. No. 209,139  
Int. Cl. B44d 1/02; H01b 5/04  
U.S. Cl. 252—63.5

8 Claims

## ABSTRACT OF THE DISCLOSURE

A resistance material including a mixture of a glass frit and finely divided particles of tantalum carbide and titanium. The resistance material is adapted to be applied to and fired on a substrate to form an electrical resistor which will readily fuse or open when subjected to an overload to prevent excessive overheating of the resistor.

## SPECIFICATION

The present invention relates to a resistance material and an electrical resistor made therefrom. More particularly, the present invention relates to a resistance material which will make a non-flammable electrical resistor.

A type of resistance material which has recently come into use is the vitreous enamel resistance material which comprises a mixture of a glass frit and finely divided particles of a conductive material. The mixture is applied to the surface of a ceramic substrate and fired. When cooled, there is provided a film of glass having the particles of the conductive material dispersed throughout the glass film. To provide a resistor of a desired resistance value, the resistance material film is generally in the form of an elongated, narrow path. Also, the resistance material film is generally coated with a plastic material to protect it from mechanical damage and from moisture and other contaminants in the atmosphere.

In the use of such vitreous enamel resistors a problem has arisen when the resistors are subjected to overload conditions. All resistors, including those made with vitreous enamel resistance materials, heat up when placed under a load in use. The higher the load the hotter the resistors will become. It has been found that resistors made with the vitreous enamel resistance materials when subjected to overload conditions heat up to such an extent that they can cause the protective coatings or other flammable material near the resistor to catch fire. To prevent such a dangerous condition from occurring, it would be desirable to have a vitreous enamel resistance material which would be self limiting as to the amount of heat it generates when subjected to overload conditions.

It is therefore an object of the present invention to provide a novel vitreous enamel resistance material and an electrical resistor made therefrom.

It is another object of the present invention to provide a vitreous enamel resistance material and a resistor made therefrom which will not excessively overheat when subjected to an overload condition.

It is still another object of the present invention to provide a vitreous enamel resistance material and a resistor made therefrom which can be made over a wide range of resistance values with stable resistance characteristics and which will not excessively overheat when subjected to an overload condition.

It is a further object of the present invention to provide a vitreous enamel resistance material and a resistor made

2

therefrom which will fuse or open to a high resistance condition when subjected to an overload condition, so as to prevent excessive overheating of the resistor.

Other objects will appear hereinafter.

5 The invention accordingly comprises a composition of matter and the product formed therewith possessing the characteristics, properties and relation of constituents which will be exemplified in the composition hereinafter described, and the scope of the invention will be indicated in the claims.

10 The drawing is a cross-sectional view, on a highly exaggerated scale, of a portion of a resistor made from the resistance material of the present invention.

15 In general, the vitreous enamel resistance material of the present invention comprises a mixture of a glass frit and finely divided particles of a mixture of tantalum carbide (TaC) and titanium (Ti). By "finely divided particles" it is meant an average particle size of not greater than about 5 microns. The mixture of the tantalum carbide and titanium is present in the resistance material in the amount of 10% to 75% by weight. The ratio of the tantalum carbide to titanium in the resistance material may be varied depending on the resistivity and temperature coefficient of resistance desired for the resistance material.

20 Increasing the amount of the tantalum carbide with respect to the amount of titanium in the resistance material will increase the resistivity and will make the temperature coefficient of resistance more positive. Thus, by adjusting the ratio of the amount of tantalum carbide to the amount of titanium and varying the amount of the conductive mixture in the resistance material, a desired temperature coefficient of resistance can be obtained at a desired resistivity of the resistance material.

25 30 35 The glass frit used in the resistance material of the present invention may be of any well known composition which has a softening point below that of the tantalum carbide and titanium. The glass frits preferably used are the borosilicate frits, such as lead borosilicate frit, bismuth, cadmium, barium, calcium or other alkaline earth borosilicate frits. The preparation of such glass frits is well known and consists, for example, of melting together the constituents of the glass in the form of the oxides of the constituents, and pouring such molten composition into water to form the frit. The batch ingredients may, of course, be any compound that will yield the desired oxides under the usual conditions of frit production. For example, boric oxide will be obtained from boric acid, barium oxide will be produced from barium carbonate, etc.

40 45 50 The coarse frit is preferably milled in a ball mill with water to reduce the particle size of the frit and to obtain a frit of substantially uniform size.

55 To make the resistance material of the present invention, commercially available tantalum carbide and titanium are each pre-milled to produce each of those materials in powdered form of the desired particle size. The tantalum carbide, titanium and glass frit in the desired proportions to achieve a resistance material of the desired resistivity and temperature coefficient of resistance are then thoroughly mixed together, such as by ball milling in water or an organic medium such as butyl carbitol acetate. After the ingredients are blended, the viscosity of the mixture is adjusted such as by removing or adding the liquid medium, to the proper viscosity for the desired manner of applying the resistance material to make a resistor.

To make a resistor with the resistance material of the present invention, the resistance material is applied in a uniform thickness on the surface of a ceramic body. The ceramic body may be comprised of any ceramic material which can withstand the firing temperature of the resistance material composition. For example, the ceramic body may be glass, alumina, steatite, porcelain, barium titanate or the like. The resistance material may be coated on the ceramic body by brushing, dipping, spraying or screen stencil application. The ceramic body and resistance material coating is then fired in a conventional furnace at a temperature at which the glass frit softens but less than the melting temperature of the tantalum carbide and titanium. The resistance material is preferably fired in a nonoxidizing atmosphere, such as argon, helium or nitrogen. When the ceramic body and resistance material are cooled, the vitreous enamel hardens to bond the resistance material to the ceramic body. When the resistance material is fired, the titanium reacts with the glass of the frit to form semiconducting suboxides of titanium,  $TiO_x$ . Thus, the conducting particles in the fired resistance material are tantalum carbide and the titanium oxide. In many cases, the titanium particles are not completely converted to the suboxides and relic titanium structures remain in the material. The starting material can also include the suboxides of titanium in place of part or all of the titanium metal to produce the resistors with the desired characteristics.

Referring to the drawing, there is shown a resistor, generally designated as 10, made from the resistance material of the present invention. Resistor 10 comprises a ceramic body 12 having a layer 14 of the resistance material coated on a surface thereof. The resistance material layer 14 comprises a glass matrix 16 having the tantalum carbide particles 18 and the  $TiO_x$  particles 20 embedded in and dispersed throughout the glass matrix 16.

Table I shows the electrical characteristics, i.e. resistance and temperature coefficient of resistance, of a number of resistors of the present invention having various total amounts of the tantalum carbide and titanium and various ratios of the tantalum carbide to titanium. The resistors were made in the manner described above, and the firing temperature and time are also shown in Table I.

TABLE I

| Weight percent of TaC and Ti | TaC/Ti (volume) | Firing conditions |            |                              | Temp. coeff. of resistance, p.p.m./° C. |          |  |
|------------------------------|-----------------|-------------------|------------|------------------------------|-----------------------------------------|----------|--|
|                              |                 | Temp., °C.        | Time, min. | Resistance, $\Omega/\square$ | -55° C.                                 | +150° C. |  |
| 25                           | 1/1             | 1,150             | 30         | 890                          | -682                                    | -507     |  |
| 25                           | 1/1             | 1,100             | 30         | 20.5K                        | -1,215                                  | -848     |  |
| 18                           | 1/1             | 1,100             | 30         | 5.0M                         | -4,233                                  | -2,110   |  |
| 67                           | 2/1             | 1,150             | 60         | 5.5                          | +150                                    | +130     |  |
| 67                           | 2/1             | 1,100             | 30         | 14                           | +73                                     | +66      |  |
| 67                           | 2/1             | 1,150             | 30         | 6                            | +89                                     | +83      |  |
| 67                           | 1/1             | 1,100             | 30         | 15                           | -100                                    | -76      |  |
| 67                           | 1/1             | 1,150             | 30         | 9                            | -144                                    | -112     |  |
| 64                           | 2/1             | 1,100             | 30         | 56                           | +20                                     | +154     |  |
| 59                           | 2.5/1           | 1,100             | 30         | 100                          | +30                                     | +28      |  |
| 49                           | 3/1             | 1,100             | 30         | 495                          | +16                                     | +9       |  |

From Table I it appears that the optimum range of tantalum carbide and titanium is between 45% and 70% by weight of the composition for producing minimized temperature coefficient of resistance characteristics for the resistors.

Table II shows the electrical characteristics of a number of resistors of the present invention made with glass frits of different compositions. In each of these resistors the total amount of tantalum carbide and titanium is 67% by weight and the ratio of tantalum carbide to titanium is 2:1 by volume. The firing conditions are shown in Table II.

TABLE II

| Glass frit                   | Firing conditions |            | Resistance, $\Omega/\square$ | Temp. coeff. of resistance |          |
|------------------------------|-------------------|------------|------------------------------|----------------------------|----------|
|                              | Temp., °C.        | Time, min. |                              | -55° C.                    | +150° C. |
| Magnesium borosilicate       | 1,100             | 30         | 14                           | +73                        | +66      |
| Do                           | 1,150             | 30         | 6                            | +89                        | +83      |
| Barium borosilicate          | 1,100             | 30         | 18                           | -188                       | -233     |
| Do                           | 1,150             | 30         | 18                           | -174                       | -188     |
| Barium boroaluminate         | 1,100             | 30         | 24                           | -718                       | -459     |
| Do                           | 1,150             | 60         | 37                           | -817                       | -581     |
| Magnesia lithia borosilicate | 1,100             | 30         | 37                           | -360                       | -242     |
| Do                           | 1,150             | 30         | 31                           | -302                       | -217     |

15

The resistors of the present invention have very good flammability characteristics in that they do not excessively overheat when subjected to an overload. This good flammability characteristic is the result of the resistors quickly converting to a high resistance condition when subjected to an overload. For example, the resistors will fuse to an open circuit condition within approximately two seconds when subjected to 40 watts, and the fusing condition occurs more quickly as the wattage increases. Thus, there is provided by the present invention a vitreous enamel resistance material and resistor made therefrom which can be provided over a wide range of resistance values, is relatively stable with regard to temperature, and has good flammability characteristics so that it will not catch fire when subjected to an overload.

It should be understood that the examples of the resistors and resistance materials of the present invention shown in Tables I and II are given merely to illustrate certain details of the invention, and are not to be taken as in any way limiting the invention thereto. The present invention may be embodied in other specific forms without departing from the spirit or essential attributes thereof, and, accordingly, reference should be made to the appended claims, rather than to the foregoing specification, as indicating the scope of the invention.

I claim:

1. A vitreous enamel resistance composition adapted to be applied to and fired on a substrate to form an electrical resistor consisting essentially of a glass frit and finely divided particles of tantalum carbide and particles containing titanium, the tantalum carbide and particles containing titanium being present in the amount of between 10% and 75% by weight.
2. A vitreous enamel resistance composition in accordance with claim 1 in which the particles containing titanium include particles of an oxide of titanium.
3. A vitreous enamel resistance composition in accordance with claim 1 in which the tantalum carbide and titanium are present in the amount of between 45% and 70% by weight.
4. A vitreous enamel resistance composition in accordance with claim 3 in which the particles containing titanium include particles of an oxide of titanium.
5. An electrical resistor having good flammability characteristics comprising a ceramic body having on a surface thereof a coating of a vitreous enamel resistor composition consisting essentially of finely divided particles of tantalum carbide and particles containing titanium embedded in a glass matrix the tantalum carbide and titanium containing particles being present in the amount of between 10% and 75% by weight.
6. An electrical resistor in accordance with claim 5 in which the particles containing titanium include particles of an oxide of titanium.
7. An electrical resistor in accordance with claim 5 in which the tantalum carbide and titanium are present in the resistor composition in the amount of between 45% and 70% by weight.

70

75

8. An electrical resistor in accordance with claim 7 in which the particles containing titanium include particles of an oxide of titanium.

|           |         |           |        |
|-----------|---------|-----------|--------|
| 2,693,521 | 11/1954 | Alexander | 117—22 |
| 3,277,020 | 10/1966 | Rao       | 252—51 |
| 3,001,893 | 9/1961  | Kreuchen  | 117—22 |
| 3,088,921 | 5/1963  | Heischman | 252—51 |

## References Cited

## UNITED STATES PATENTS

5 ALFRED L. LEAVITT, Primary Examiner

M. F. ESPOSITO, Assistant Examiner

U.S. Cl. X.R.

|           |        |                 |         |                                 |
|-----------|--------|-----------------|---------|---------------------------------|
| 3,441,516 | 4/1969 | Milligan et al. | 106—49  |                                 |
| 3,394,087 | 7/1968 | Huang et al.    | 106—48  |                                 |
| 3,180,841 | 4/1965 | Murphy          | 252—516 |                                 |
| 2,851,376 | 9/1958 | Adlassnig       | 106—48  | 10 106—48, 49; 117—221; 252—516 |
| 3,503,801 | 3/1971 | Huang et al.    | 117—221 |                                 |